

# UNITED STATES PATENT OFFICE.

EARL V. WAGNER, OF SCRANTON, PENNSYLVANIA, ASSIGNOR TO THE WAGNER FIRE  
BRICK COMPANY, OF HELENA, MONTANA.

## COMPOSITION OF MATTER FOR MAKING FIRE-BRICK.

1,198,171.

Specification of Letters Patent. Patented Sept. 12, 1916.

No Drawing.

Application filed January 8, 1916. Serial No. 70,983.

*To all whom it may concern:*

Be it known that I, EARL V. WAGNER, a citizen of the United States, residing at Scranton, in the county of Lackawanna and State of Pennsylvania, have invented a new and useful Composition of Matter for Making Fire-Brick, of which the following is a specification.

My composition consists of the following 10 named ingredients combined in substantially the proportions here stated:

Coal ash ----- 100 lbs.  
Magnesia ----- 3 lbs.  
Water ----- 2 to 2½ gals.

15 It is not intended to confine the patent here applied for to the use of the ingredients specified in the proportions stated, as the proportions may in some cases be advantageously varied, producing substantial 20 identity of result. To illustrate: If the fusion point of the coal ash is found to be less than 2600 degrees Fahrenheit, or if a high fusion point for the fire brick is 25 desired, the percentage of magnesia used is to be increased. Thus, taking 100 pounds of coal ash as a basis whose fusion point is 2600 degrees Fahrenheit, to this is added 3 pounds of magnesia which will raise the 30 fusion point of the mixture to 3250 (3225-3275) degrees Fahrenheit. If on account of impurities and foreign substances in the coal ash its fusion point is found to be below 2600 degrees Fahrenheit, the percentage of magnesia must be correspondingly increased to produce the above named 35 result, the percentages being based upon the original fusion point of the coal ash and upon the fusion point of the fire brick which 40 it is desired to obtain. The proportions

above stated are therefore approximately pure coal ash having a fusion point of approximately 2600 degrees Fahrenheit.

Grind and mingle the coal ash with the magnesia, then add the water and mix until 45 thoroughly plastic. Press the plastic mass through a molding machine of approved type. Cut the brick to the size desired by the use of a cutting machine of approved type. The freshly cut bricks are then re- 50 pressed in a repressing machine of approved type in which they are subjected to heavy pressure sufficient to fill out all angles and decrease the laminations and to strengthen the bond. Then place the brick in a closed 55 drying oven and dry for six to eight hours at a temperature of 500-600 degrees Fahrenheit. Remove the bricks while hot to a closed burning kiln whose temperature is gradually raised to 2200-2400 degrees 60 Fahrenheit at which temperature the bricks are fired for seven to eight days when they are allowed to cool gradually, resulting in the finished product.

I am not aware that the ingredients aforesaid, in the proportions stated, or in any other proportions, or at all, have ever been used for any purpose prior to my invention and discovery thereof.

What I claim is:

The herein described composition of matter for making fire brick, consisting of coal ash, 100 pounds; magnesia, 3 pounds; water, two to two and one-half gallons, substantially as described.

EARL V. WAGNER.

Witnesses:

HOMER C. HUTCHINS,  
DAVID J. JONES.

Copies of this patent may be obtained for five cents each, by addressing the "Commissioner of Patents, Washington, D. C."